

Patented Sept. 4, 1945

2,384,002

# UNITED STATES PATENT OFFICE

2,384,002

## LUBRICANT

Alfred L. Bayes, Kenmore, N. Y., assignor to Carbide and Carbon Chemicals Corporation, a corporation of New York

No Drawing. Application June 9, 1943,  
Serial No. 490,174

8 Claims. (Cl. 252—47)

This invention relates to lubricants, and particularly to mineral oil lubricants having incorporated therein minor quantities of additive material adapted to improve lubrication properties, and to inhibit or retard metal corrosion and deterioration of the oil in normal lubrication service.

Commercial petroleum lubricating oils, as originally extracted and refined, may have certain corrosiveness toward metals. Oils which are not initially corrosive may become so under conditions of use in an internal combustion engine, where oxidation, under high temperature and pressure, usually effects certain break-down in the oil, which promotes or creates corrosive conditions, as well as other deteriorating influences. In modern automotive engines the bearing metals often are cadmium-silver, cadmium-nickel or copper-lead alloys, and these alloys are especially susceptible to corrosion in contact with mineral lubricating oils. The problem of inhibiting the corrosive action of oils on metal surfaces, and of retarding deterioration of the oil through oxidation, is, therefore, of essential importance, and to avoid these difficulties the addition of inhibitors to lubricating oils has become a common practice.

It is an object of this invention to provide new and improved oil additive materials, which are adapted in very small concentrations to impart to lubricating oil, and maintain therein, substantially non-corrosive characteristics toward common bearing metals, while at the same time producing in the oil a greater resistance to deterioration through oxidation. A further object is to provide improved mineral oil lubricants incorporating such additives.

The inhibitor additives proposed by the invention are materials formed by mixture of two components, one a dimorpholine sulfide or polysulfide composition and the other the compound mercaptobenzothiazole. The dimorpholine derivatives which are suitable may be further described as compositions of the characteristic structure:



in which  $x$  represents one or more sulfur atoms. Individual compounds of this structure, like dimorpholine monosulfide or dimorpholine disulfide are satisfactory for the purpose intended, as are also products comprising mixtures of the

polysulfides, including the trisulfide, tetrasulfide or higher derivatives.

Dimorpholine monosulfide, with the sulfur linkage



can be prepared by the reaction of morpholine and sulfur dichloride in an inert solvent such as benzene. The pure product is a white crystalline material which is soluble in most organic solvents, and has a melting point of about 112° C. The reaction of sulfur monochloride with morpholine produces the sulfur linkage



or dimorpholine disulfide. This compound is also a white crystalline solid, containing 27.1% sulfur and having a melting point of about 123° C. A product comprising mixtures of the polysulfide derivatives can be made by reacting morpholine with elemental sulfur in the presence of lead oxide or other metal oxide catalyst; and by modification in the mol proportions of the reactants used, in the quantity and purity of the catalyst, or in the temperature of the reaction, compositions of different sulfur content can be obtained, with the sulfur varying, for example, within the range of about 32% to 42%. The melting point of these reaction mixtures is not sharply defined, although the products usually melt within the range of 75° C. to 85° C., with the melting temperature decreasing as the sulfur content increases. Also with increase in sulfur content, the recovered solid products vary from white to yellow in color.

In the inhibitor mixture here proposed, the dimorpholine sulfide component will function primarily as an anti-oxidant, and in association with mercaptobenzothiazole a cooperative, further improved, corrosion inhibiting and anti-oxidant action is attained. The latter compound is particularly effective as a corrosion protective agent for copper-containing metals, and it provides in addition the joint effect of an increased inhibitor life with regard to both anti-oxidant and corrosion protective functions. Mercaptobenzothiazole alone is not readily soluble in lubricating oil, but when carefully and thoroughly blended with a dimorpholine sulfide component, the resulting product can be incorporated into oil without difficulty in required inhibitive amounts. In a preferred method of blending the two components the mercapto-

benzothiazole is dissolved in the melted dimorpholine sulfide composition, and this fused product has advantages in the compounding with oil. There is some indication that chemical combination may occur in such a mixture, but whether or not this is the case, the results intended by the invention can be accomplished with either a mechanically mixed or fused product. Where the additive is defined as a mixture, blending of the two components in either manner is intended.

The most effective concentrations of the new additives will vary with different lubricating oils, and with specific lubricating conditions, but for most purposes a range of from 0.10% to 2.0% by weight of total additive will be found satisfactory. The individual components may be present in equal weight proportions, particularly when fused mixtures are used, but in many instances predominating amounts of the dimorpholine sulfide will be found desirable. For example, in proportions of 0.5% of the dimorpholine sulfide, with 0.05%, 0.1% or 0.2% of mercaptobenzothiazole, excellent results have been attained, and a fused mixture of equal parts of each component, with a total additive amount of 0.2% by weight, has in some oils produced a marked inhibitor improvement.

Test results on representative embodiments of the invention are shown in the following table, wherein there are indicated property changes in oil, both with and without the new additive, as effected by operation for 36 hours in a Chevrolet engine. A commercial Mid-Continent solvent refined oil of viscosity S. A. E. 20 was used in these tests. The additive represented by MS is a dimorpholine polysulfide mixture, as previously described, having a sulfur content of about 39%, and MBT is an abbreviation for mercaptobenzothiazole. In one instance the additive was a simple mixture of the two components, and in the second test a fused product, in parts by weight as indicated, was used.

| Additive          | 36 hour Chevrolet engine test |                       |                                    |
|-------------------|-------------------------------|-----------------------|------------------------------------|
|                   | Copper lead bearing wt. loss  | Increase in viscosity | Increase in neutral No. Mg.KOH/gm. |
| None              | Grams 0.711                   | Percent 262           | 6.2                                |
| 0.5% MS, 0.1% MBT | 0.057                         | 19.2                  | 0.51                               |
| 0.5% (6:1 MS-MBT) | 0.073                         | 31.4                  | 0.32                               |

The protective action for bearing metals afforded by the new additives is obvious from the above results, and that oil deterioration is also retarded can be readily seen by the fact that the change in viscosity and neutralization number is of a substantially lower degree in the inhibited oil. The same relative results have been obtained with additive mixtures of other proportions, and with those containing different morpholine derivatives within the class described. The invention contemplates usage of these new additives in any of the common petroleum lubricating oils, including both asphaltic and paraffin base oils, and it does not preclude the further addition of detergents, oiliness agents, or other property-modifying materials, if desired.

This application contains subject matter in common with my copending application Serial No. 470,213, filed December 26, 1942, issued as Patent No. 2,351,657 on June 20, 1944.

I claim:

1. A lubricant comprising a mineral oil containing corrosion and oxidation inhibiting amounts of an additive mixture composed of mercaptobenzothiazole and a dimorpholine sulfide of the structure:



wherein  $x$  is at least one.

2. A lubricant comprising a mineral oil containing corrosion and oxidation inhibiting amounts of an additive composed of a fused mixture of mercaptobenzothiazole and a dimorpholine sulfide of the structure:



wherein  $x$  is at least one.

3. A lubricant comprising a mineral oil containing corrosion and oxidation inhibiting amounts of an additive composed of a fused mixture of mercaptobenzothiazole and a mixture of dimorpholine sulfides of the structure:



wherein  $x$  is at least one and represents a sulfur content in the sulfide mixture of from about 32% to 42%.

4. A lubricant comprising a petroleum lubricating oil containing an additive mixture composed of about 0.05% to 0.20% by weight of mercaptobenzothiazole, and about 0.5% of dimorpholine sulfides of the structure:



wherein  $x$  is at least one.

5. A lubricant comprising a petroleum lubricating oil containing about 0.2% to 1.0% of an additive composed of a fused mixture in equal parts by weight of mercaptobenzothiazole and a mixture of dimorpholine sulfides of the structure:



wherein  $x$  is at least one and represents a sulfur content in the sulfide mixture of from about 32% to 42%.

6. Method of lubricating bearing surfaces composed of metal having the corrosion susceptibility of copper-lead and cadmium-silver alloys, which comprises applying to the bearing surfaces a lubricant having incorporated therein, in corrosion-inhibiting amounts, an additive mixture composed of mercaptobenzothiazole and a dimorpholine sulfide of the structure:



wherein  $x$  is at least one.

7. Method of lubricating bearing surfaces composed of metal having the corrosion susceptibility of copper-lead and cadmium-silver alloys, which comprises applying to the bearing surfaces

a lubricant having incorporated therein an additive mixture composed of about 0.05% to 0.20% by weight of mercaptobenzothiazole, and about 0.5% of dimorpholine sulfide of the structure:



5

wherein  $x$  is at least one.

8. Method of lubricating bearing surfaces composed of metal having the corrosion susceptibility of copper-lead and cadmium-silver alloys, which comprises applying to the bearing surfaces a lu-

bricant having incorporated therein an additive composed of a fused mixture in equal parts by weight of mercaptobenzothiazole and a mixture of dimorpholine sulfides of the structure:



wherein  $x$  is at least one and represents a sulfur content in the sulfide mixture of from about 32% to 42%.

ALFRED L. BAYES.